

1

2,931,774

## LUBRICANT STABILIZED BY BIS ALKYLENE PYROBORATE

Glenn E. Irish, Detroit, Mich., assignor to Ethyl Corporation, New York, N.Y., a corporation of Delaware

No Drawing. Application May 3, 1956  
Serial No. 582,606

3 Claims. (Cl. 252—49.6)

This invention relates to improved hydrocarbon lubricants and more particularly to hydrocarbon lubricants stabilized by a bis alkylene pyroborate.

Hydrocarbon lubricants deteriorate when subjected to the elevated temperatures encountered in lubrication service. This deterioration leads to deleterious deposits of carbonaceous material on the lubricated surfaces which greatly reduce the effectiveness of the lubricant.

It is, therefore, an object of this invention to provide improved hydrocarbon lubricants. Another object is to provide improved hydrocarbon lubricants containing stable esters of pyroboric acid. A further object of this invention is to provide improved hydrocarbon lubricants having a high degree of thermal stability. Another object is to provide an improved crankcase lubricating oil containing a bis alkylene pyroborate.

The above and other objects of this invention are accomplished by providing a hydrocarbon lubricant containing a stabilizing amount of boron as a bis alkylene ester of pyroboric acid. The resulting lubricant has a greatly enhanced thermal stability. Pyroboric acid may be represented by the formula:



and the corresponding bis alkylene esters have the formula:



where R is an alkylene group of from 2 to 6 carbon atoms in length and which contains from 2 to about 20 carbon atoms. Thus, R can represent a substituted alkylene group of from 2 to 6 carbon atoms in length which contains alkyl, aryl, cycloalkyl, aralkyl, alkaryl, halogen, ketone, carboxyl, or other substituents. These substituents may contain up to 18 carbon atoms when the alkylene group contains two carbon atoms, but substituents having up to about 8 carbon atoms are preferred as they give an ester of lower molecular weight, and thus more boron per mole. Alkyl substituents of from 1 to 6 carbon atoms are particularly preferred because the esters containing these groups are more easily prepared.

When a bis alkylene pyroborate is compounded with a crankcase lubricating oil, it is desirable to add a small amount, i.e., sufficient bis alkylene pyroborate to form a composition containing from 0.001 to 1.0 weight percent of boron. However, a preferred embodiment of this invention comprises a crankcase lubricating oil containing from about 0.01 to about 0.15 weight percent boron as a bis alkylene pyroborate as it has been found that these amounts of boron effectively increase the thermal stability. A particularly preferred embodiment of this invention comprises a liquid hydrocarbon crankcase lubricating oil containing from 0.01 to 0.15 weight percent boron as bis(2-methyl-2,4-pentylene) pyroborate.

2

The bis alkylene pyroborate esters used in the practice of this invention may be prepared from boric acid,  $\text{H}_3\text{BO}_3$ , and an aliphatic diol, by first converting the boric acid to metaboric acid, HOBO, and then reacting the metaboric acid with an equimolar amount of the diol under conditions such that 1.5 moles of water are removed from the reaction mixture for each mole of diol reacted.

The process of preparing bis alkylene pyroborates is carried out in an appropriate solvent which is inert to both the reactants and products of the reaction and which forms a minimum boiling azeotrope with water. These solvents ordinarily have boiling points of from 80° C. to the decomposition temperatures of the reactants and products of the reaction. Appropriate solvents include aliphatic and aromatic hydrocarbons and organic compounds containing elements other than carbon and hydrogen. Examples of suitable solvents include toluene, benzene, xylene, dioxane and cyclohexane.

Further embodiments of this invention are illustrated by the following examples in which all parts are by weight unless otherwise stated.

## EXAMPLE I

## Preparation of metaboric acid

Two hundred parts of toluene and 61.8 parts of boric acid,  $\text{H}_3\text{BO}_3$ , were added to a reaction vessel equipped with heating means, stirring means and reflux distillation means. The vessel was then heated with stirring to the boiling point of the toluene-water azeotrope. Heating and agitation were continued until an amount of the azeotrope corresponding to 18 parts of water had been removed from the reaction mass. The vessel which contained a solution of metaboric acid, HOBO, in toluene, was then cooled.

## EXAMPLE II

To the toluene-metaboric acid solution prepared in Example I, containing 43.8 parts of HOBO, was added 118.2 parts of 2-methyl-2,4-pentanediol. The resulting mixture was again heated with stirring to the boiling temperature of the toluene water azeotrope until an amount of azeotrope corresponding to 27 parts of water had been removed from the reaction mass. The remaining toluene was removed by distillation at atmospheric pressure leaving a water-white liquid having a boiling point of 114 to 115° C. at 2 millimeters of mercury. The molecular weight of this product was determined to be 267 and on analysis the product was found to have 54.6% of carbon, 9.2% hydrogen, 8.12% boron and, by difference, 28.01% oxygen. This corresponds to a calculated analysis of 53.4% carbon, 8.96% hydrogen, 8.02% boron and 29.62% oxygen and a calculated molecular weight of 269.95 for bis(2-methyl-2,4-pentylene) pyroborate having the formula:



The refractive index of this compound is  $1.43180 n_{\text{D}}^{20}$ .

## EXAMPLE III

Seventy-six parts of propylene glycol were added to a toluene-metaboric acid solution, prepared as described in Example I, and reacted according to the procedure described in Example II. The reaction was discontinued after an amount of toluene-water azeotrope corresponding to 27 parts of water had been removed from the reaction vessel. On removing the toluene by atmospheric

## 3

distillation, 143 parts of bis propylene pyroborate, a water-white liquid, remained in the reaction vessel.

## EXAMPLE IV

The procedure of Example III is followed except that 118 parts of hexanediol-2,5 is reacted with metaboric acid in lieu of propylene glycol, to prepare bis(2,5-hexylene) pyroborate.

## EXAMPLE V

Following the procedure of Example II, 104.1 parts of pentanediol-1,5 is reacted with 43.8 parts of metaboric acid to prepare bis(1,5-pentylene) pyroborate.

## EXAMPLE VI

A solution of metaboric acid and xylene was prepared from 61.8 parts of boric acid and 215 parts of xylene according to the procedure in Example I. To this solution is added 62 parts of ethylene glycol and the mixture is heated until an amount of xylene water azeotrope, amounting to 27 parts of water, is removed. Atmospheric distillation of the remaining xylene enables recovery of a good yield of bis ethylene pyroborate.

The lubricants which are beneficially enhanced by the practice of this invention include those fractions or blends of fractions from mineral oils which are used for lubricating and related purposes. Lubricating oil stock is usually considered to include all the distillate obtainable from crude oils after the lower boiling fractions and gas oils have been expelled, as well as some of the residues that are left in the still when non-asphaltic crudes are distilled.

Generally, lubricating oils are made from distilled fractions of a crude, but often these distilled fractions are combined with refined residuum, such as bright stocks, to yield oils having excellent lubricating qualities.

Lubricating oils are made into literally thousands of products which may consist of the pure mineral oils or blends containing one or more other ingredients. Among these products are motor oils, aviation oils, machine oils, transformer oils, cable oils, turbine oils, cutting oils, loom oils, textile oils, etc. Greases are lubricating oils which have been rendered solid or semi-solid by the addition of soaps or similar materials. Typical embodiments of this invention comprising a bis alkylene pyroborate and a hydrocarbon lubricant are illustrated by the following examples.

## EXAMPLE VII

To 500 parts of a commercially available neutral crankcase lubricating oil was added 2.8 parts of bis(2-methyl-2,4-pentylene) pyroborate, a quantity sufficient to produce a composition containing about 0.05 weight percent boron. The mixture was agitated until the bis(2-methyl-2,4-pentylene) pyroborate was completely dispersed in the oil.

## EXAMPLE VIII

To 10,000 parts of a wholly-distilled mixed base, solvent refined lubricating oil having a gravity of 28.9° API, a viscosity grade of SAE 10W-20 and a viscosity index of 135.7 is added 2.75 parts of bis(1,5-hexadecalene) pyroborate and the mixture is stirred until the pyroborate is dissolved in the oil.

## EXAMPLE IX

To 1000 parts of a mixed base solvent-refined lubricating oil containing bright stock and which has an SAE viscosity grade of 20, an API gravity of 30.5° and a viscosity index of 107.4, is added 16.75 parts of bis(1,5-pentylene) pyroborate.

## EXAMPLE X

To 2162 parts of a wholly distilled lubricating oil having an API gravity of 30.3°, a viscosity index of 154.2 and an SAE number of 5W-20, is added 1.6 parts of

## 4

bis ethylene pyroborate and the mixture is stirred until the ester is dissolved.

## EXAMPLE XI

5 To 216 parts of a wholly distilled lubricating oil having an API gravity of 29.1, an SAE number of 10W-30 and a viscosity index of 138.9, is added 21.4 parts of bis(3-methyl-1,3-butylene) pyroborate. The mixture is agitated until the pyroborate has dissolved.

## EXAMPLE XII

To 1,000 parts of the oil described in Example VII is added 15 parts of bis(1,2-eicosylene) pyroborate and the mixture is agitated until the pyroborate is dissolved.

## EXAMPLE XIII

To 1,000 parts of the oil described in Example VIII is added 10 parts of bis(1,6-hexylene) pyroborate.

## EXAMPLE XIV

20 To a lubricating grease consisting of 11 parts of aluminum stearate, 1 part of lithium stearate and 88 parts of an oil having a viscosity of 100 seconds Saybolt Universal at 100° F., is added 2 parts of bis(2-methyl-2,4-pentylene) pyroborate and the mixture is blended until the ester is completely dispersed through the grease.

25 To demonstrate the superiority of a crankcase lubricating oil of this invention containing a bis alkylene pyroborate, comparative tests were run on the oil prepared according to Example VII and the identical oil which did not contain any bis(2-methyl-2,4-pentylene) pyroborate. These oils were compared by the Panel Coker Test which measures the oxidative stability of a lubricating oil at a hot metal surface. This test is described in the Aeronautical Standards group of the departments of Navy and Air Force specification MIL-L-7808c dated November 2, 1955. In this instance the tests were run at 550° F. The results of the tests are summarized in Table I. These data illustrate that a lubricating oil containing a small amount of a bis alkylene pyroborate has a greatly reduced coking tendency at elevated temperature when compared to an identical oil containing none of the pyroborate esters. Thus, the oil containing a pyroborate ester has a greatly enhanced thermal stability and a superior resistance to oxidative deterioration.

TABLE I  
Panel coker test

| Additive                                              | Milligrams of Deposit |
|-------------------------------------------------------|-----------------------|
| None                                                  | 468                   |
| 0.05% Boron as bis(2-methyl-2,4-pentylene) pyroborate | 312                   |

55 In addition to the bis alkylene pyroborates, the hydrocarbon lubricants of this invention may contain other additives. These other additives may include for example, viscosity index improvers, detergents, corrosion inhibitors, metal deactivators, rust inhibitors, color stabilizers, pour depressants, emulsifiers, dyes, etc., and in the case of greases metallic soaps, fillers, etc.

60 The diols suitable for use in preparing the pyroborate esters of this invention include those wherein the hydroxyl groups are separated by from 2 to 6 carbon atoms. Examples of the pyroborate esters which are prepared from these diols include: bis ethylene pyroborate, bis(1,3-propylene) pyroborate, bis(1,4-butylene) pyroborate, bis(1,5-pentylene) pyroborate, bis(1,2-heptylene) pyroborate, bis(1,3-butylene) pyroborate, bis(1-methyl-1,2-propylene) pyroborate, bis(1,3 - pentylene) pyroborate, bis(2,5-hexylene) pyroborate, bis(2-methyl-2,4-pentylene) pyroborate, bis(2-methyl-4,4-diethyl-1,2-pentylene) pyroborate, bis(6-n-propyl-1,4-nonylene) pyroborate, bis(1,2-eicosylene) pyroborate, bis(3,5-diethyl-3,5-hexylene) pyroborate, bis(2-chloro-3,5-pentylene) pyroborate, bis-

(2-benzyl-3,5-pentylene) pyroborate, bis 2-(p-carboxyl-phenyl)-3,6-hexylene pyroborate, bis (3,5-dihexylphenyl-ethylene) pyroborate, etc.

I claim:

1. A hydrocarbon lubricant containing from about 0.001 to about 1.0% of boron as a liquid bis alkylene pyroborate having the formula



10

wherein R is an alkylene group of 2 to 6 carbon atoms in length and containing 2 to about 20 carbon atoms.

2. An improved liquid hydrocarbon crankcase lubricating oil containing from about 0.001 to about 1.0% of boron as a liquid bis alkylene pyroborate having the formula



20

wherein R is an alkylene group of 2 to 6 carbon atoms in length and containing 2 to about 20 carbon atoms.

3. An improved liquid hydrocarbon crankcase lubricating oil containing from about 0.001 to about 1.0% of boron as liquid bis (2-methyl-2,4-pentylene) pyroborate having the formula



References Cited in the file of this patent

UNITED STATES PATENTS

|           |          |               |
|-----------|----------|---------------|
| 2,721,181 | Lawrence | Oct. 18, 1955 |
| 2,741,548 | Darling  | Apr. 10, 1956 |
| 2,795,548 | Thomas   | June 11, 1957 |